

Feb. 19, 1974

J. KANDLER ET AL

3,793,228

DETERGENT COMPOSITIONS CONTAINING MALEIC ACID VINYL  
ALCOHOL COPOLYMERS AS BUILDERS

Original Filed Sept. 16, 1970

2 Sheets-Sheet 1

Fig.1.

% WK = *Cleansing Power Quotient*



Concentration of Surface Active Substance: 0.4 g/Liter 100%  
Alkylarylsulfonate  
0.15 g/Liter Pluronic®

Curve 1 : Vinyl Alcohol/Maleate; Molecular Proportion 1:1  
Curve 2 : Styrene / Maleate; Molecular Proportion 2:1  
Curve 3 : Styrene / Maleate; Molecular Proportion 2.5:1

Feb. 19, 1974

J. KANDLER ET AL

3,793,228

DETERGENT COMPOSITIONS CONTAINING MALEIC ACID VINYL  
ALCOHOL COPOLYMERS AS BUILDERS

Original Filed Sept. 16, 1970

2 Sheets-Sheet 2

Fig. 2.

*% WK = Cleansing Power Quotient*



Curve 1 : Vinyl Alcohol/Maleate; Molecular Proportion 1:1  
Curve 2 : Styrene/Maleate; Molecular Proportion 2:1  
Curve 3 : Styrene/Maleate; Molecular Proportion 2.5:1

1

3,793,228

DETERGENT COMPOSITIONS CONTAINING  
MALEIC ACID VINYL ALCOHOL COPOLY-  
MERS AS BUILDERS

Joachim Kandler and Karl Merkenich, Cologne, Herbert Landgraber, Efferen, near Cologne, Klaus Henning, Hurth, near Cologne, and Alfred Kohlkamp, Hofheim, Taunus, Germany, assignors to Knapsack Aktiengesellschaft, Knapsack, near Cologne, Germany

Original application Sept. 16, 1970, Ser. No. 72,705, now abandoned. Divided and this application Oct. 24, 1972, Ser. No. 299,821

Claims priority, application Germany, Oct. 8, 1969,

P 19 50 702.9

Int. Cl. C02b 5/06; C08f 15/02; C11d 3/20

U.S. Cl. 252—541

7 Claims

## ABSTRACT OF THE DISCLOSURE

Builders for detergent and cleaning agents. The builders are comprised of water-soluble salts of cotelomers or copolymers of vinyl alcohol with maleic acid.

This application is a division of application Ser. No. 72,705, filed Sept. 16, 1970, now abandoned.

The present invention provides builders for detergent and cleaning agents, the builders comprising organic polymer compounds.

It has already been reported that the cleaning power of soaps and synthetic detergents in detergent and cleaning compositions can be improved by means of certain addends. These cleaning intensifiers are termed builders. Detergent and cleaning compositions having such builders therein are more effective, yet less costly than corresponding formulations which are free from builders.

The mechanism and the details of the "builder effect" have not yet been fully described. Vital to the function of the builder is a plurality of processes comprising, for example: the stabilization of pigment dirt suspensions; the emulsification of dirt particles; the effect on the surface and interfacial properties of aqueous surfactant solutions; the solubilization of water-insoluble ingredients of the cleaning bath; the peptization of agglomerated dirt; the neutralization of acid substances; and the inactivation of mineral matter in the cleaning bath.

To determine the quality and qualification of individual materials for use as a builder, it is good practice to test their behavior and efficiency in washing or cleaning operations, to ensure the qualitative and quantitative determination of all factors that make their contribution to the builder effect.

Classical builders comprise water-soluble inorganic alkali metal salts, such as alkali metal carbonates, borates, phosphates, polyphosphates, bicarbonates, and silicates.

While a plurality of materials have been suggested for use as builders, the fact remains that linear condensed phosphates or polyphosphates, more particularly pentasodium triphosphate or sodium tripolyphosphate, are almost exclusively used as the builders in customary detergent and cleaning compositions, having up to substantially 50 weight percent builder therein. Despite the many advantages which polyphosphate builders offer over further conventional builders, they have been found during their long years practical use to also have some disadvantages.

In all polyphosphates, the P—O—P bond, which is formed by dehydration, is relatively easy to split hydrolytically. This results in the formation of decomposition products, such as metaphosphates or orthophosphate of reduced efficiency, particularly in the case of liquid detergent and cleaning compositions, but also in the spray process. In addition thereto, liquid detergent formulations may be

2

rendered turbid, or precipitation may occur therein, which is undesirable.

The considerably increased consumption of phosphate-containing detergent and cleaning agents both for domestic and industrial purposes has also effected an increase in the phosphate content of natural waters receiving phosphate salt-containing waste water. On discussing the eutrophication of waters, which has been found to occur at constantly increasing rates for some years, the nitrates and phosphates have recently been held to have properties that are able under certain conditions to promote the growth of certain alga species, and thereby to make their contribution to the eutrophication of water. Even though it is impossible for the time being definitely to clarify this problem, it is highly desirable to have potential substitutes for the builders, namely tripolyphosphate, that find widespread use in current detergent formulations. These substitutes are intended to avoid eutrophication of waters.

Organic compounds having builder properties have also been disclosed more recently. Water-soluble salts of amino-polycarboxylic acids, for example, the sodium salt of ethylene diamine tetracetic acid, or of amino- and hydroxylalkylidene phosphonic acids have more particularly been suggested for use as builders. These materials have substantially not been put to commercial use, and they also contain a good deal of nitrogen and phosphorus atoms.

In U.S. Pat. 3,308,067, it has been suggested that water-soluble alkali metal, ammonium and substituted ammonium salts of homopolymers and copolymers of aliphatic polycarboxylic acids be used as builders in detergent and cleaning compositions. The comonomers include primarily short chain olefins and unsaturated carboxylic acids. Representatives of these builders, which are termed polyelectrolyte builders, include for example, the sodium salt of polymaleic acid or copolymers of propylene or styrene with maleic acid. These builders either have no satisfactory builder properties or are too costly for mass production.

The present invention now unexpectedly provides water-soluble salts of cotelomers or copolymers of vinyl alcohol with maleic acid, which can be used with particular advantage as builders in detergent and cleaning compositions. The builders suggested to be used in accordance with the present invention preferably have the following general formula:



in which

*m* is the maleic acid fraction in the copolymer, of at most about 55 mole percent,

Me stands for an alkali metal or ammonium ion, and *n* is a whole number within a range of which the lower limit is 3 and of which the upper limit is defined by the solubility of the polymer in water,

In accordance with a further feature of the present invention, the copolymer builders have a preferred molecular weight of between 1,500 and 3,000. In accordance with a still further feature of the present invention, the maleic acid fraction in the copolymer or cotelomer should preferably be limited to a value of between about 25 and 50 mol percent.

To produce detergent and cleaning compositions, it is possible to introduce the copolymer builders of the present invention into conventional detergent and cleaning agent formulations, such as those which are based on ion-active and/or non-ionic surfactants, and which may be

tionally be used in combination with further addends. In accordance with the present invention, the builder is generally used in a proportion of between about 10 and 80 weight percent, preferably between about 15 and 60 weight percent, based on the dry substance of the detergent and cleaning agent. In addition to a water-soluble copolymer of vinyl alcohol and maleic acid, the detergent and cleaning agents may contain an alkali metal polyphosphate as a further builder. Detergent and cleaning compositions prepared in accordance with the present invention give a pH-value of between 8 and 12 in the aqueous medium of the wash bath.

The addends, which may be present together with the ion-active and/or non-ionic surfactants in the detergent formulation, comprise substances, such as sodium silicate, magnesium silicate, sodium sulfate, sodium perborate, optical brighteners, carboxymethyl cellulose and/or enzymes, for example.

The builders of the present invention are produced in conventional manner, for example, by subjecting a copolymer or telomer of maleic anhydride and vinyl acetate to saponification by means of a sodium hydroxide solution.

The properties of the builders of the present invention can be evaluated, for example, in dispersing tests. Starting with an aqueous suspension, which contained either hydrophilic particles, such as iron (III) oxide, or hydrophobic particles, for example graphite particles, it was possible by the addition of the builders of the present invention to produce stable dispersions. This is demonstrated in the table hereinafter. As results from the tabulated test results, the builder substances of the present invention can be said to have the properties required of a builder. On comparing Table 1 with Table 2, it will readily be seen that hydrophilic dirt particles are particularly well dispersed by a vinyl alcohol/maleate cotelomer. The reason for this is that both the settling rate and sedimentation volume are smaller than in a comparative test made with the use of a styrene/maleate cotelomer as the builder. As compared with conventional alkali metal tripolyphosphate builders, those of the present invention have the advantage of dispersing hydrophobic dirt, whereas the alkali metal tripolyphosphates fail to produce such effect.

#### EXAMPLE 1

The sodium salt of a vinyl alcohol/maleic acid copolymer was tested as to its dispersing effect in an aqueous suspension of 4 weight percent graphite powder at various pH-values, and the effect produced was compared with that produced by a conventional styrene/maleic acid copolymer builder, in a corresponding suspension. The settling times of the graphite particles in 25 cc. mixing cylinders, and the volume of sedimentation were determined in each case as an index of the dispersing effect. The builder was used in the suspension in a concentration of 0.1 weight percent, based on the aqueous solution. The results obtained are summarized in Table 1 below.

TABLE 1

| Builder | Settling time in hours |       | Volume of sedimentation in cubic centimeters |       |
|---------|------------------------|-------|----------------------------------------------|-------|
|         | pH 8                   | pH 10 | pH 8                                         | pH 10 |
| A-----  | 21                     | 21    | 1.9                                          | 1.8   |
| B-----  | 24                     | 24    | 1.9                                          | 1.8   |
| C-----  | 20                     | 20    | 3.5                                          | 3.4   |

NOTE.—A=Styrene/maleate; molar ratio=2:1; molecular weight=1,330. B=Styrene/maleate; molar ratio=2.5:1; molecular weight=1,544. C=Vinyl alcohol/maleate; molar ratio=1:1; molecular weight=1,940.

#### EXAMPLE 2

The procedure was the same as that described in Example 1 save that iron (III) oxide powder with a particle size of less than 0.058 mm. was substituted for the

graphite powder. The test results are indicated in Table 2 below.

TABLE 2

| Builder | Settling time in hours |       | Volume of sedimentation in cubic centimeters |       |
|---------|------------------------|-------|----------------------------------------------|-------|
|         | pH 8                   | pH 10 | pH 8                                         | pH 10 |
| A-----  | 20                     | 23    | 1.3                                          | 1.2   |
| B-----  | 23                     | 26    | 1.3                                          | 1.2   |
| C-----  | 28                     | 36    | 1.1                                          | 1.0   |

NOTE.—A=Styrene/maleate; molar ratio=2:1; molecular weight=1,330. B=Styrene/maleate; molar ratio=2.5:1; molecular weight=1,544. C=Vinyl alcohol/maleate; molar ratio=1:1; molecular weight=1,940.

#### EXAMPLE 3

15 Wash tests were made to determine the cleansing power quotients of wash liquors which for a constant concentration of surface active substance contained varying proportions of builder (invention), and the test results obtained were graphically plotted in FIG. 1 of the accompanying graphs (curve 1). Analogous wash tests with the use of conventional builders, such as styrene/maleate, were made for the purpose of comparison.

16 The cleansing power quotients are also graphically plotted in FIG. 1, curves 2 and 3.

25 The wash tests were made on standard cotton fabrics soiled with "Krefeld" dirt in a "Launder-O-meter" at a wash bath temperature of 95° C. Standard fabrics soiled with Krefeld dirt have been defined by Kurt Lindner in the book entitled: "Tenside, Textilhilfsmittel-Waschrohstoffe," Wissenschaftl. Verlagsgesellschaft Stuttgart (1964), volume II, page 1837.

30 The wash water had a hardness of 20° (German degrees of hardness) and a pH of 10. The wash period was 30 minutes and the bath ratio, expressed by the ratio of material to be washed in kg. to wash liquor in liter was 1:50, and the wash operation was carried out in the presence of 10 steel balls. The wash liquor contained a 100% alkylaryl sulfonate as a surface-active substance as well as Pluronic®, which is a non-ionic polyoxypropylene glykol.

35 After the prescribed wash time, the standard cotton fabric was rinsed, once hot and once cold, and its degree of whiteness was then determined using an Elrepho remission photometer (a produce of Zeiss) and a filter R 55.

40 Based on the test result obtained, the cleansing power quotient was calculated along the following formula:

$$\text{Percent WK} = \frac{\text{Percent } WG_g - \text{Percent } WG_b}{\text{Percent } WG_u - \text{Percent } WG_b} \cdot 100$$

45 in which

Percent WK=Percent cleansing power,  
Percent  $WG_g$ =Percent whiteness of washed fabric,  
Percent  $WG_b$ =Percent whiteness of unwashed fabric,  
Percent  $WG_u$ =Percent whiteness of unsoiled fabric.

50 As can be seen from curves 1, 2 and 3 shown in FIG. 1, more cleansing power is imparted to the wash liquor by the builder of the present invention, to which belongs curve 1, than by conventional builders, to which belong curves 2 and 3.

#### EXAMPLE 4

55 The procedure was the same as that described in Example 3, save that the wash liquor contained the builder and a fully active detergent composed of:

|                         | G./liter |
|-------------------------|----------|
| Sodium silicate         | 0.2      |
| Magnesium silicate      | 0.2      |
| Soap                    | 0.15     |
| Sodium perborate        | 1.0      |
| 50% alkylaryl sulfonate | 1.0      |
| Non-ionic substances    | 0.1      |
| Carboxymethyl cellulose | 0.2      |

75 As can be seen from curve 1 in FIG. 2, the builder of the present invention was again found to distinguish

favorably over conventional builders (cf. curves 2 and 3).

What is claimed is:

1. A detergent composition based on anionic surfactants, nonionic surfactants, or mixtures thereof, and containing, as a builder, from 10 to 80 weight percent based on the dry weight of the composition of a water soluble salt of a copolymer of vinyl alcohol and maleic acid having the following formula:



in which

*m* is the maleic acid fraction in the copolymer and is from about 25 to 55 mole percent,

Me stands for an alkali metal or ammonium ion, and

*n* is a whole number with a range of which the lower limit is 3 and of which the upper limit is defined by the solubility of the polymer in water.

2. A detergent composition as claimed in claim 1 wherein in the copolymer of vinyl alcohol and maleic acid is present in an amount between about 15 and 60 weight percent based on the dry weight of the detergent composition.

3. A detergent composition in accordance with claim 1, wherein the copolymer has a molecular weight of between 1,500 and 3,000.

4. A detergent composition according to claim 1 wherein maleic acid constitutes 50 mole percent of the copolymer.

5. A detergent composition in accordance with claim 1, further containing an effective amount of an alkali metal polyphosphate as a supplemental builder.

6. A detergent composition according to claim 1, producing a pH value of between 8 and 12 in an aqueous wash or cleaning liquor.

10 7. A detergent composition in accordance with claim 1, further containing a minor amount of at least one material selected from the group consisting of sodium silicate, magnesium silicate and sodium sulfate.

#### References Cited

#### UNITED STATES PATENTS

|              |         |           |          |
|--------------|---------|-----------|----------|
| 3,700,599    | 10/1972 | Mizuno    | 252—99   |
| 3,686,145    | 8/1972  | Haschke   | 260—67 U |
| 3,676,373    | 7/1972  | Paviak    | 252—531  |
| 20 3,627,686 | 12/1971 | Sabatelli | 252—527  |
| 3,579,455    | 5/1971  | Sabatelli | 252—135  |
| 3,308,067    | 3/1967  | Diehl     | 252—89 X |
| 3,284,364    | 11/1966 | Siegele   | 252—132  |
| 2,306,071    | 12/1942 | McNally   | 260—78   |
| 25 2,047,398 | 7/1936  | Voss      | 260—2    |

LEON D. ROSDOL, Primary Examiner

D. L. ALBRECHT, Assistant Examiner

U.S. Cl. X.R.

252—89, 132, 135, 180, 523, Digests 2, 11; 260—78.5 R